

March 14, 1944.

W. J. CROOK

2,343,888

HEAT TREATMENT OF STEEL

Filed April 8, 1942

2 Sheets-Sheet 1



*Fig. 1*

WD2340 Steel

Hot Rolled

1000X Picral Etch



*Fig. 2*

WD2340 Steel

Normalized 1800°F-3hr

1000X Picral Etch



*Fig. 3*

WD2340 Steel

Normalized 1800°F-3hr

Drawn 1100°F - 3hr

1000X Picral Etch

Winton J. Crook

Inventor

By G. J. Tessman and J. H. Church

Attorneys

March 14, 1944.

W. J. CROOK

2,343,888

HEAT TREATMENT OF STEEL

Filed April 8, 1942

2 Sheets-Sheet 2



*Fig. 4*

WD2340 Steel

Hot Rolled

1000X Picral Etch



*Fig. 5*

WD2340 Steel

Normalized 1800°F-3hr

1000X Picral Etch



*Fig. 6*

WD2340 Steel

Normalized 1800°F. - 3hr.

Drawn 1100°F. - 3hr.

1000X Picral Etch

Winton J. Crook

Inventor

By G.J. Tessmanich - J.H. Church

Attorneys

## UNITED STATES PATENT OFFICE

2,343,888

## HEAT TREATMENT OF STEEL

Welton J. Crook, United States Army,  
Davenport, Iowa

Application April 8, 1942, Serial No. 438,102

1 Claim. (Cl. 148—21.5)

(Granted under the act of March 3, 1883, as  
amended April 30, 1928; 370 O. G. 757)

The invention described herein may be manufactured and used by or for the Government for governmental purposes, without the payment to me of any royalty thereon.

The present invention relates to the heat treatment of steel, both plain and alloy, and more particularly to a new and improved method of enhancing the physical properties of "abnormal" steel by means of a special heat treating process.

As is well known in the art, the operation of normalizing consists in heating steel to some temperature above the upper critical temperature and below 2000° F., for a time sufficient to produce a state of solid solution of all contained carbides, followed by cooling in still air. This procedure is commonly applied to heavy forgings, steel castings and similar products, principally for the purpose of homogenizing the metal. It is also applied to rolled sections generally as a preliminary treatment which is followed by heating, quenching and drawing. Normalizing followed by reheating below the lower critical temperature is also well known as a method of removing cooling stresses produced by normalization.

Heretofore, where the properties required in steel were above those normally obtained in the "as rolled" or "as cast" state, the steel has generally been subjected to heat treatment by heating the same to some temperature above the upper critical limit, quenching in oil or water and then reheating to some temperature below the critical point, the reheating or draw treatment being adjusted with reference to the particular properties desired. This quench and draw procedure, while of definite value in improving the properties of the steel, is nevertheless characterized by certain disadvantages. Thus, for example, the quenching operation produces somewhat variable results depending on the mass of the object being treated, particularly where the object has sections of widely different sizes, in which cases uniformity of results is

exceedingly difficult if not impossible to attain. Moreover, the machinability of the ultimate product is not all that could be desired. Again, the usual treatment of quench and draw often results in the development of residual stresses which appear after partial or finish machining, especially in objects which require a high degree of straightness or dimensional stability. Warpage is also undesirably high as a result of the quench and draw operation, and, lastly, considerable equipment is required by the prior art processes.

One of the objects of the present invention is to provide a new and improved process of enhancing the physical properties of steel, which obviates the foregoing disadvantages of the prior art quench and draw process.

Another object is a process of the character described wherein the uniformity of the results obtained is not adversely affected either by the configuration or by the mass of the article being treated.

A further object is a heat treating process which permits the attainment of a given set of enhanced physical properties and especially Brinell hardness or its equivalent, together with a greatly superior machinability in the ultimate product, compared to the machinability of a product of comparable physical properties produced by the prior art quench and draw procedure.

A still further object is a process of the character hereinbefore indicated, which eliminates to a high degree the presence of residual stresses and warpage tendency typical of steel objects which have been treated by the usual quench and draw process.

Another object is to provide a steel of improved physical properties, characterized by high yield strength and superior machinability.

Other objects will be apparent as the invention is hereinafter more fully described.

The foregoing objects may be accomplished in accordance with the present invention, one

aspect of which comprises a special heat treating process applicable to any steel, whether plain carbon or alloy, which exhibits a condition of substantial abnormality under the condition of the McQuaid-Ehn test. In accordance with the present invention, such abnormal steel is first normalized and thereafter drawn at a temperature below the lower critical temperature thereof and within the range of approximately 500° F. to approximately 1200° F. The thus treated steel is characterized by an enhanced yield strength and superior machinability, as herein-after more particularly pointed out.

The present invention is based on the discovery that, when operating under certain conditions and upon a class of steel which may conveniently be designated as "reactive," a draw treatment following a normalizing operation produces an altogether unanticipated and thus far inexplicable enhancement of the physical properties of the treated steel, rather than the expected impairment thereof. Indeed, when a steel of a "reactive" type is normalized and then subjected to a reheating treatment below the lower critical temperature, for example, at 500° F., 600° F. and up to about 1000° F., it has been found that the higher the reheating temperature, the higher the enhancement in the yield point of the product, thereby affording a method of controlling the degree of enhancement desired in respect to yield strength.

"Reactive" steels as hereinbefore briefly indicated, comprise any steel, whether plain carbon or alloy, which exhibits a condition of substantial "abnormality" under the McQuaid-Ehn test. Such a steel characteristically possesses after normalization a so-called "molybdenum" structure under microscopic examination, and preferably, but not necessarily, should have a McQuaid-Ehn grain size rating (A. S. T. M.) of from about six to about eight. Such steels when normalized assume a characteristic fine-grained acicular ferrite structure wherein the carbide particles are rejected at the grain boundaries. "Abnormal" steel possessing the foregoing characteristics exhibits the peculiar property, not possessed by "normal" steel, of responding favorably to a normalize and draw treatment as hereinafter described; i. e., the yield strength of the "abnormal" steel is thereby enhanced, whereas the physical properties of "normal" steel, on the other hand, are either unaffected or impaired.

In carrying out the process of the present invention, a "reactive" steel is first normalized in any convenient manner well known to the art, i. e., it is heated to some temperature, above the upper critical limit and below a temperature of about 2000° F., for a time sufficient to produce a state of solid solution of all contained carbides, and then cooled freely in still air. The second part of the treatment comprises a drawing operation, wherein the normalized "reactive" steel is reheated to a temperature below the lower critical temperature and within the range of approximately 500° F. to approximately 1200° F., preferably from about 600° F. to about 1000° F. It will thus be apparent that the process requires no special apparatus, and may be simply and readily carried out with less equipment than that required for the usual quench and draw process.

In order more clearly to disclose the nature of the present invention several specific examples will hereinafter be described. It should be understood, however, that this is done solely by way of example, and is not to be construed as a

limitation upon the spirit or scope of the appended claim.

When a "reactive" steel is normalized and thereafter subjected to a reheating treatment below the critical temperature and within the range of from about 500° F. up to approximately 1000° F., it has been found that the higher the draw temperature, the greater the enhancement in the yield point. This effect of the draw temperature may be seen by reference to Table I.

TABLE I

*Effect of normalizing and draw temperature on abnormal WD2340 steel*

| Norm. temp. | Draw temp. | Tens. str. | Yield str. | Elongation percent 2" | Red. area | Brinell hardness |
|-------------|------------|------------|------------|-----------------------|-----------|------------------|
| °F.         | °F.        | P. s. t.   | P. s. t.   |                       | Percent   |                  |
| 1,650       | 500        | 111,500    | 71,500     | 21.2                  | 52.2      | 229              |
| 1,650       | 700        | 111,000    | 72,250     | 20.0                  | 49.4      | 229              |
| 1,650       | 900        | 111,500    | 75,250     | 22.5                  | 53.3      | 229              |
| 1,650       | 1,100      | 102,500    | 67,500     | 23.0                  | 57.3      | 197              |
| 1,800       | 600        | 111,000    | 70,250     | 19.6                  | 51.3      | 223              |
| 1,800       | 700        | 111,250    | 71,500     | 21.2                  | 50.5      | 223              |
| 1,800       | 900        | 111,000    | 75,000     | 21.0                  | 51.3      | 212              |
| 1,800       | 1,100      | 102,500    | 70,000     | 24.2                  | 56.2      | 212              |

If the draw temperature materially exceeds about 1000° F. (for example, above about 1200° F.) there is, in many cases, a diminution in yield strength of the normalized and drawn "reactive" steel. However, there is also a corresponding increase in elongation and reduction of area, and therefore, in practice, the draw temperature may in some instances be desirably carried as high as 1100° F., for example, in order to attain a selected combination of physical properties.

In the case of a "non-reactive" steel (e. g., one which is substantially "normal" under the conditions of the McQuaid-Ehn test), the same normalize and draw procedure which produces enhanced physical properties in a "reactive" steel, results in many instances in an impairment of yield strength in normalized and drawn "non-reactive" steel. The striking difference in the response of "reactive" and "non-reactive" steel to a normalize and draw treatment is illustrated by the data given in Table II.

TABLE II

|                                                  | Tensile str. | Yield str. | Elong. percent in 2" | Red. area | Brinell hardness |
|--------------------------------------------------|--------------|------------|----------------------|-----------|------------------|
| REACTIVE                                         |              |            |                      |           |                  |
| Steel A—<br>As received.....                     | P. s. t.     | P. s. t.   |                      | Percent   |                  |
| As rolled.....                                   | 113,800      | 67,000     | 16.1                 | 34.0      | 223              |
| Same after<br>1,800° F. norm.<br>1,100° F. draw. | 104,800      | 75,250     | 22.2                 | 52.5      | 207              |
| NON-REACTIVE                                     |              |            |                      |           |                  |
| Steel B— as re-<br>ceived.....                   | 100,500      | 59,000     | 23.6                 | 48.3      | 197              |
| Same after<br>1,800° F. norm.<br>1,100° F. draw. | 98,750       | 58,000     | 22.7                 | 47.4      | 207              |
| Steel C— as re-<br>ceived.....                   | 114,000      | 66,400     | 19.5                 | 37.8      | 217              |
| Same after<br>1,800° F. norm.<br>1,100° F. draw. | 107,500      | 65,000     | 22.0                 | 53.5      | 217              |

Referring now to the six figures of the accompanying drawings.

Figs. 1 to 3 are reproductions of photomicrographs of a typical normal, "non-reactive"

WD2340 steel, as rolled (Fig. 1), normalized (Fig. 2) and normalized and drawn (Fig. 3).

Figs. 4 to 6 are similar views of a typical abnormal "reactive" WD2340 steel, as rolled (Fig. 4), normalized (Fig. 5) and normalized and drawn (Fig. 6).

Figs. 1 to 3 shows clearly that no useful reaction has taken place in the case of the normal steel, whereas Figs. 4 to 6 illustrate the changes effected in an abnormal steel by the steps of the herein described process. The chemical analysis of the two steels shown in Figs. 1 to 6 were very closely similar as far as carbon, manganese, phosphorus, sulfur, silicon and nickel are concerned. The "reactive" steel, however, showed spectrographic traces of aluminum, whereas the "non-reactive" steel did not.

The manner in which the condition of "abnormality" in a "reactive" steel is produced or brought about forms no part of the present invention, inasmuch as any suitable procedure, well known in the prior art, may be used for this purpose. Thus, for example, the condition may be created by suitable aluminum additions to the steel. Other grain-control adjuncts may also be used, either singly or in combination, if desired. Where aluminum is employed, however, there are several reasons why neither a definite aluminum addition can be specified nor a definite percentage of residual aluminum oxide can be required in a finished steel in order to assure that condition of substantial abnormality which provides the convenient index of "reactivity" herein employed. In the first place, the effect of definite aluminum additions to steel for purpose of grain size control depends largely on the particular melting practice employed and is greatly influenced by the state of deoxidation of the metal before the aluminum is added. In other words, different melting practices may require more or less aluminum to produce a given degree of grain size control. Moreover, the amount of aluminum oxide remaining in grain size controlled steel is generally exceedingly small and an accurate chemical analysis with respect thereto is difficult to obtain. For these and other reasons, the specification of a given grain size range is a more reliable and indeed more fundamental means of assuring "reactivity" in steel than any attempt to specify either the amount or character of the grain size control adjunct available to the steelmaker for the purpose of attaining the required condition of substantial abnormality. In short, in the procurement of a "reactive" steel, it is preferable to leave it to the steel maker to attain a specified grain size according to his particular furnace practice, and not to limit his choice of grain size control procedures available to him.

In the case of certain steels containing molybdenum, it has been observed that the herein described normalize and draw procedure will effect a slight improvement in physical properties even when the steel is only partly abnormal. However, substantial improvement in yield strength is generally attained only in steels exhibiting a condition of substantial abnormality under the McQuaid-Ehn test. For these reasons, the preferred "reactive" steel has a grain size rating of, say, from six to eight (A. S. T. M.).

#### EXAMPLES

In order still more clearly to illustrate the broad principles of the present invention, several specific examples will now be described in detail.

The chemical analysis, maker's name, "WD number" (War Department specification number), physical properties developed by each steel when normalized at 1800° F. and drawn at 1100° F. are shown in Tables III and IV.

TABLE III  
Chemical composition of McQuaid-Ehn test samples

| Specimen No. | C    | Mn   | P       | S       | Ni      | Cr      | Mo.     |
|--------------|------|------|---------|---------|---------|---------|---------|
| 15           |      |      | Percent | Percent | Percent | Percent | Percent |
| 1-52         | 0.40 | 0.69 | 0.016   | 0.015   | 3.44    |         |         |
| 1-58A        | 0.42 | 0.74 | 0.016   | 0.014   | 3.52    |         |         |
| 1-59A        | 0.40 | 0.95 |         |         | Trace   | 1.20    | 0.25    |
| 1-59B        | 0.38 | 0.86 |         |         | Trace   | 0.82    | 0.22    |
| 1-60A        | 0.45 | 0.78 | 0.011   | 0.018   | 3.53    |         |         |
| 1-61A        | 0.43 | 0.73 |         |         | 3.66    |         |         |
| 1-61B        | 0.40 | 0.71 |         |         | 3.55    |         |         |
| 20           |      |      |         |         |         |         |         |
| 1-62A        | 0.40 | 0.71 | 0.015   | 0.018   | 3.40    |         |         |
| 1-62B        | 0.40 | 0.70 | 0.015   | 0.017   | 3.34    |         |         |
| 1-63A        | 0.39 | 0.73 | 0.016   | 0.014   | 3.44    |         |         |
| 1-63B        | 0.44 | 0.79 | 0.017   | 0.010   | 3.61    |         |         |
| 2-4A         | 0.40 | 0.69 | 0.016   | 0.016   | 3.44    |         |         |
| 2-5A         | 0.44 | 0.73 | 0.018   | 0.017   | 3.47    |         |         |
| 2-6A         | 0.38 | 0.70 | 0.017   | 0.017   | 3.51    |         |         |
| 25           |      |      |         |         |         |         |         |
| 2-8B         | 0.38 | 0.67 | 0.015   | 0.008   | 3.68    |         |         |
| 2-9          | 0.39 | 0.75 | 0.014   | 0.013   | 3.47    |         |         |
| 2-15A        | 0.55 | 0.81 | 0.018   | 0.010   |         | 0.83    | 0.15    |
| 2-16B        | 0.41 | 0.81 | 0.020   | 0.019   |         | 0.99    | 0.21    |
| 2-17A        | 0.48 | 0.74 | 0.008   | 0.020   |         | 0.94    | 0.19    |
| 2-17B        | 0.46 | 0.53 | 0.015   | 0.009   | 1.70    | 1.05    |         |

TABLE IV  
Description of samples subjected to McQuaid-Ehn test

| Spec. No. | Maker             | W.D. No. | Physical ten. str. | Prop. yield str. | Norm. and drawn   |       |         |
|-----------|-------------------|----------|--------------------|------------------|-------------------|-------|---------|
|           |                   |          |                    |                  | Elong. percent 2" | R. A. | Brinell |
| 40        |                   |          |                    |                  |                   |       |         |
| 1-52      | Rep. <sup>1</sup> | 2340     | P. s. i.           | P. s. i.         | 23.7              | 55.9  | 207     |
| 1-58A     | Rep.              | 2340     | 103,500            | 77,500           | 20.4              | 51.9  | 207     |
| 1-59A     | Tim. <sup>2</sup> | 4140     | 112,750            | 84,500           | 19.3              | 55.7  | 212     |
| 1-59B     | Rep.              | 4140     | 111,000            | 80,500           | 19.2              | 55.1  | 207     |
| 1-60A     | Car. <sup>3</sup> | 2340     | 113,500            | 83,000           | 19.5              | 37.8  | 217     |
| 1-61A     | Rep.              | 2340     | 114,000            | 66,500           | 23.8              | 54.1  | 207     |
| 1-61B     | Rep.              | 2340     | 105,500            | 75,500           | 23.2              | 55.9  | 207     |
| 1-62A     | Rep.              | 2340     | 105,750            | 77,000           | 20.5              | 49.1  | 217     |
| 1-62B     | Rep.              | 2340     | 104,000            | 80,250           | 22.2              | 55.1  | 207     |
| 1-63A     | Rep.              | 2340     | 111,500            | 70,000           | 19.0              | 45.4  | 223     |
| 1-63B     | Cop. <sup>4</sup> | 2340     | 109,500            | 79,500           | 22.8              | 56.2  | 228     |
| 2-4A      | Rep.              | 2340     | 103,500            | 77,500           | 23.7              | 55.9  | 207     |
| 2-5A      | Rep.              | 2340     | 108,750            | 75,000           | 25.3              | 58.5  | 223     |
| 2-6A      | Rep.              | 2340     | 101,250            | 71,000           | 22.9              | 55.1  | 196     |
| 2-8B      | Rep.              | 2340     | 98,750             | 66,000           | 22.7              | 47.4  |         |
| 2-9       | Rep.              | 2340     | 103,750            | 78,250           | 22.8              | 56.7  | 202     |
| 2-15A     | Car.              | 4150     | 126,500            | 93,000           | 15.7              | 46.2  | 269     |
| 2-16B     | Car.              | 4140     | 119,500            | 83,000           | 18.9              | 50.2  | 228     |
| 2-17A     | Tim.              | 4150     | 121,250            | 87,250           | 17.6              | 45.4  | 255     |
| 2-17B     |                   | 3240     | 124,500            | 70,500           | 19.0              | 58.6  | 235     |

<sup>1</sup> Republic.

<sup>2</sup> Timken.

<sup>3</sup> Carnegie.

<sup>4</sup> Copperweld.

In performing the McQuaid-Ehn test, samples of each of these steels were box carburized for eight hours at 1700° F. and cooled in the box in the furnace. The rate of cooling from the carburizing temperature was regulated so that at least three hours were taken in cooling through the transformation range so that distinct carbide grain boundaries would be formed in the hypereutectoid zone.

The results of the McQuaid-Ehn tests are shown in Table V. In this table, under the heading "Reaction to normalize and draw" the steels which were "reactive" to treatment at 1800° F. normalization followed by an 1100° F. draw are rated "yes" where they met or exceeded the properties listed in Table VI.

TABLE V  
Results from McQuaid-Ehn tests

| Spec. No. | WD number | Normality rating | Reaction to normalize and draw | Grain size rating | A. S. T. M. No. |
|-----------|-----------|------------------|--------------------------------|-------------------|-----------------|
| 1-59A     | 4140      | A                | Yes                            | 5                 |                 |
| 1-59B     | 4140      | A                | Yes                            | 5                 |                 |
| 2-5B      | 2340      | A                | No                             | 2                 |                 |
| 2-17A     | 4150      | A                | No                             | 3                 |                 |
| 1-60A     | 2340      | A                | Yes                            | 12-6              |                 |
| 2-5A      | 2340      | B                | Yes                            | 8                 |                 |
| 1-63B     | 2340      | B                | Yes                            | 15-7              |                 |
| 2-16B     | 4140      | B                | Yes                            | 15-7              |                 |
| 1-52      | 2340      | B                | Yes                            | 4                 |                 |
| 1-58A     | 2340      | B                | Yes                            | 7                 |                 |
| 2-4A      | 2340      | B                | Yes                            | 6                 | 15              |
| 1-62A     | 2340      | B                | Yes                            | 7                 |                 |
| 1-62B     | 2340      | B                | Yes                            | 6                 |                 |
| 1-61A     | 2340      | B                | Yes                            | 8                 |                 |
| 1-61B     | 2340      | B                | Yes                            | 6                 |                 |
| 2-6A      | 2340      | B                | Yes                            | 17-3              |                 |
| 2-9       | 2340      | B                | Yes                            | 7                 |                 |
| 2-17B     | 3240      | B                | Yes                            | 8                 |                 |
| 1-63A     | 2340      | C                | Yes                            | 8                 |                 |
| 2-15A     | 4150      | C                | Yes                            | 7                 |                 |

<sup>1</sup> Duplex.

TABLE VI  
Limiting properties to be developed in normalized and drawn steels

| Steel                | Tens. str.          | Yield str.         | Elong. percent 2" | Red. area     |
|----------------------|---------------------|--------------------|-------------------|---------------|
| WD 2340 <sup>1</sup> | P. s. i.<br>100,000 | P. s. i.<br>70,000 | 18                | Percent<br>30 |
| WD 4140 <sup>2</sup> | 105,000             | 80,000             | 18                | 30            |

<sup>1</sup> Including WD1040, 3140 and 3240 steels.

<sup>2</sup> Including WD4150 steel.

From an inspection of Table V it will be evident that a "reactive" steel is preferably one having a McQuaid-Ehn grain size rating of from six to eight.

In general, steels which do not contain molybdenum must be "partly abnormal" or "abnormal" in order to assure the so called "molybdenum" structure when normalized, and this structure has been found to be characteristic of all steels which are "reactive" to the normalize and draw treatment. In the case of steel which contain molybdenum (for example WD4140 steels), slight "reactivity" is noted in some cases, even where the steel is normal or only partly abnormal. It is probable, however, that a degree of abnormality must exist in all steels if they are to respond favorably to the normalize and draw treatment. In other words, a condition of substantial abnormality is correlated with substantial "reactivity" within the meaning of the present invention, lesser degrees of abnormality being correlated with lower degrees of "reactivity."

Numerous advantages are realized by the practice of the present invention. Thus, for example, the process of the present invention is easier to apply than the usual process of quench and draw, and requires less equipment. Moreover, when various sections or sizes of material are to be treated, the effect of mass on the uniformity

of the results obtained does not intervene as it does in the quench and draw treatment of the prior art.

A further important advantage of the herein described process as compared to the quench and draw process, relates to the machinability of the ultimate product. It has been found in numerous tests that, for a given set of physical properties and especially Brinell hardness or its equivalent, the machinability obtained by the present process is greatly superior to that obtained by a quench and draw treatment. This improvement may be illustrated by a test performed on two sets of five inch steel bars selected from the same heat of "abnormal" WD2340 steel, one set being heat treated by oil quenching and drawing, the other set being treated in accordance with the present invention, both having the same hardness, namely, 286 Brinell. Both sets of bars were then drilled in a vertical Stecher drill. On the average, it required three (3) drill blades to drill each of the oil quenched and drawn bars, whereas one blade was capably drilling three (3) of the normalized and drawn bars.

Another advantage of the present invention was noted in the machining of objects requiring a high degree of straightness or dimensional rigidity, as for example, in the case of rods and tubes for gun recoil mechanism. It was found that the normalize and draw treatment eliminated to a high degree the development of residual stresses which often results after partial or finish machining of similar objects which have been quenched and drawn. It was also noted that warpage in steel which has been treated by normalize and draw is greatly decreased and practically eliminated.

In the foregoing detailed description of the present invention it will be apparent to those skilled in the art that many variations may be made without departing from the spirit and scope thereof. I therefore intend to be restricted only in accordance with the following patent claim.

I claim:

The two-step process of producing steel gun recoil cylinders, counter-recoil cylinders, hollow control rods, and the like, which comprises the steps of normalizing said steel, and thereafter drawing said normalized steel below the lower critical temperature thereof and within the range of approximately 500° F. to approximately 1200° F., said steel being selected from the group exhibiting a condition of substantial abnormality under the conditions of the McQuaid-Ehn test and having a grain size rating (A. S. T. M.) of from six to eight, inclusive, whereby the physical properties of said steel are enhanced without impairing the machinability thereof by hard spots due to the formation of martensitic structure and whereby stress relieving operations are substantially eliminated due to the absence of distortion.

WELTON J. CROOK.

**Certificate of Correction**

Patent No. 2,343,888.

March 14, 1944.

WELTON J. CROOK

It is hereby certified that error appears in the printed specification of the above numbered patent requiring correction as follows: Page 3, second column, lines 35 to 40 inclusive, the heading to Table IV should appear as shown below instead of as in the patent—

| Physical prop. norm. and drawn |       |        |                |                 |                                      |               |     |
|--------------------------------|-------|--------|----------------|-----------------|--------------------------------------|---------------|-----|
| Spec. No.                      | Maker | WD No. | Ten. str. psi. | Yield str. psi. | Elong. percent<br>$2^{\prime\prime}$ | R. A. percent | BHN |
|                                |       |        |                |                 |                                      |               |     |

and that the said Letters Patent should be read with this correction therein that the same may conform to the record of the case in the Patent Office.

Signed and sealed this 6th day of June, A. D. 1944.

[SEAL]

**LESLIE FRAZER,**  
*Acting Commissioner of Patents.*